# EUROPEAN PATENT SPECIFICATION

(11) **EP 3 320 544 B1**
(45) Date of publication and mention of the grant of the patent: **31.03.2021**
(21) Application number: 16736567.5
(22) Date of filing: 29.06.2016
(51) Int. Cl.: H01F 1/057, H01F 41/02, C22C 38/00

(54) **MAGNET**
MAGNET
AIMANT

(30) Priority: 06.07.2015 GB 201511821
(43) Date of publication of application: 16.05.2018
(73) Proprietor: Dyson Technology Limited, Malmesbury, Wiltshire SN16 0RP (GB)
(72) Inventor: CELIK, Tuncay, Malmesbury Wiltshire SN16 0RP (GB)
(74) Representative: Hobday, Duncan Stuart
(86) International application number: PCT/GB2016/051944
(87) International publication number: WO 2017/006082

(56) References cited:
- EP-A1- 2 131 474
- EP-A1- 2 254 131
- EP-A1- 2 790 193
- US-A1- 2005 208 218

## Description

The present invention relates to a rare earth magnet and a method of making a rare earth magnet. More specifically, the present invention relates to a rare earth magnet with improved coercivity and a method of making the same.

Rare earth magnets may comprise a crystal lattice structure containing grains of rare earth alloys. It has been shown that the magnetic properties, particularly the coercivity, of such magnets can be improved by substituting dysprosium or terbium into the crystal lattice structure. Dysprosium or terbium can be substituted either into the bulk of the crystal lattice, for instance via a binary addition, or along the grain boundaries of the crystal lattice via a heat-treatment step, such as grain boundary diffusion. Diffusion of dysprosium or terbium along the grain boundaries is preferred as less dysprosium or terbium is required to achieve the same improvements in magnetic properties, such as coercivity.

For grain boundary diffusion, dysprosium or terbium must be deposited on the rare earth magnet for effective substitution to occur. The high price and low natural abundance of dysprosium and terbium however has meant that recent research efforts have focussed on providing an improved magnet using smaller amounts of dysprosium or terbium. A problem with these deposition techniques is that a considerable amount of time may be required to deposit the dysprosium or terbium, and that wastage of expensive dysprosium or terbium can still occur. It is also considered that some dysprosium containing materials used in current deposition techniques, for example DyF₃, may be detrimental to the magnetic properties of the substrate. A method of depositing dysprosium or terbium onto a rare earth magnetic substrate that is fast and/or materially efficient without having a detrimental effect on the magnetic properties of the substrate is desired. EP 2 131 474 A1 discloses a method of depositing Dy or Tb by spray methods, before diffusing the film into the magnet.

In a first aspect, the present invention provides a magnet comprising a magnetic body and a layer of dysprosium; wherein the magnetic body contains grains of a rare earth magnet alloy, and the layer of dysprosium is deposited onto the surface of the magnetic body by a cold spray process. This intermediate product is specified in claim 7.

The grains of rare earth alloy may include magnetic alloys that contain samarium, praseodymium, cerium or neodymium. Of specific interest are sintered alloys containing neodymium or samarium alloys, particularly Nd₂Fe₁₄B, SmCo₅ and Sm(Co, Fe, Cu, Zr)₇.

The use of cold spray to deposit a layer of dysprosium onto the magnetic body has several advantages over conventional techniques. For example, dysprosium metal can be used directly in the process instead of dysprosium rich powders, such as DyF₃ or Dy₂O₃. As mentioned above, fluoride slurries may be detrimental to the magnetic properties of the magnetic substrate. Where a powder rich in Dy₂O₃ is used, dysprosium oxide can remain after heat-treatment or further sintering of the magnet, leading to inefficient substitution of dysprosium into the lattice structure. These undesired side-effects may be overcome by cold spraying dysprosium metal instead of dysprosium oxides directly onto the magnetic body.

Conventional deposition techniques, such as dysprosium vapour-sorption and dip coating, require a large amount of time and controlled conditions to produce a rare earth magnet with sufficient levels of dysprosium substitution. In contrast, with a cold spray process a less controlled environment is possible and the deposition process is relatively rapid, with dysprosium deposition taking a matter of seconds. Additionally, since standard conditions may be used in cold spray, less of the dysprosium metal is oxidised during processing, thereby providing a better quality of dysprosium for diffusion within the magnetic body.

The amount of dysprosium deposited on the magnetic body can also be carefully controlled and specifically targeted using cold spray. Conventional deposition techniques can lead to unpredictable amounts of deposition and also a high wastage of expensive dysprosium metal that is deposited in the wrong areas.

The magnetic body may be sintered. A sintered magnetic body allows for better grain boundary diffusion to occur. A degree of sintering can take place during the grain boundary diffusion heat-treatment. However it is more beneficial if the magnetic body has been pre-sintered prior to the cold spray deposition of the dysprosium layer. A pre-sintered magnetic body means that a separate heat-treatment step is required for diffusing the dysprosium into the body. This separate heat-treatment step can be carefully tuned so that a grain boundary diffusion is dominant over a full diffusion of dysprosium into the alloy grains.

During heat treatment an amount of dysprosium may be diffused within the grains. A smaller amount of diffused dysprosium can improve the coercivity of the magnetic body compared with increasing the initial amount of dysprosium in the grains. Furthermore, the amount of diffusion can be controlled and tuned by varying the conditions of heat treatment, i.e. temperature ramp up, holding time and temperature, cooling rates and gas atmosphere. The grains may contain an amount of diffused dysprosium of between 0.5 to 15 percent by weight and the dysprosium can be diffused along the boundaries of the grains to form a shell layer.

The grains may comprise a neodymium alloy. Neodymium alloys have a favourable magnetic strength and are widely used in applications where a strong permanent magnet is required. Examples of such applications include electric motors and generators. For some applications the operating temperature can exceed 150 °C. The coercivity of conventional neodymium magnets however can suffer at elevated temperatures. It has been found that substituting an amount (typically as much as 12%) of neodymium for dysprosium in the crystal lattice can significantly increase coercivity and improve the performance of the magnet at elevated temperatures. The neodymium alloy may be Nd₂Fe₁₄B which exhibits a particularly improved magnet. It is believed that this improvement is due to Dy₂Fe₁₄B and (Dy,Nd)₂Fe₁₄B having a higher anisotropy field than Nd₂Fe₁₄B.

The Nd₂Fe₁₄B alloy magnet may comprise grains of Nd₂Fe₁₄B with a shell layer comprising Dy₂Fe₁₄B or (Dy,Nd)₂Fe₁₄B, the shell layer having a thickness of about 0.5 µm. The deposited dysprosium diffuses through the magnetic body during a heat-treatment after depositing the cold sprayed layer of dysprosium on the magnetic body. During the heat-treatment, the deposited dysprosium substitutes with neodymium atoms along the grain boundaries of the crystal lattice, instead of permeating throughout the bulk of the crystal lattice. The shell layer of the grains produced by cold spray and heat-treatment can be much thinner compared to magnets produced by other methods. The shell layer can have a thickness of 0.5 µm. Therefore a much higher concentration of dysprosium is present at the grain boundaries, meaning that less dysprosium is needed to achieve the same coercivity enhancement that is exhibited in conventional dysprosium substituted rare earth magnets.

The deposition thickness of the layer of dysprosium may be between 1 to 5 µm. This thickness results in effective grain boundary diffusion during heat treatment and also reduces wastage of expensive dysprosium. The continuous layer of dysprosium should have an average thickness of 1 to 5 µm since a layer with a uniform thickness is not required.

In a second aspect, the present invention provides a method of manufacturing a magnet, the method comprising: providing a magnetic body containing grains of a rare earth alloy; cold spray depositing a layer of dysprosium onto the surface of the magnetic body to form a magnet; and heat-treating the magnet. The method is specified in claim 1.

Heat-treating the magnet may comprise a grain boundary diffusion process. More specifically, heat-treating the magnet may comprise: heating the magnet to a first elevated temperature; cooling the magnet to second elevated temperature; and quenching the magnet to room temperature. This process can be conducted such that the first elevated temperature may be at least 900 °C. Independent of the first temperature, the second elevated temperature may be at least 500 °C. In addition to the temperatures, the magnet may be held at the first elevated temperature for at least 6 hours.

Independent of the time that the magnet is held first temperature, the magnet may be held at the second elevated temperature for at least 0.5 hours. These temperatures and times are particularly favoured as they provide good diffusion conditions without the grains undergoing sintering or further sintering.

In a third aspect, the present invention provides a magnet comprising a magnetic body and a layer of terbium; wherein the magnetic body contains grains of a rare earth magnet alloy, and the layer of terbium is deposited onto the surface of the magnetic body by a cold spray process. This intermediate product is also specified in claim 7.

In a fourth aspect, the present invention provides a method of manufacturing a magnet, the method comprising: providing a magnetic body containing grains of a rare earth alloy; cold spray depositing a layer of terbium onto the surface of the magnetic body to form a magnet; and heat-treating the magnet. This method is also specified in claim 1.

In order that the present invention may be more readily understood, an embodiment of the invention will now be described, by way of example, with reference to the accompanying drawings, in which:
Figure 1 shows a cross-sectional schematic representation of a magnet of the present invention; and
Figure 2 is a flowchart showing the manufacturing process of the magnet of the present invention.

The magnet 1 of Figure 1 comprises a magnetic body 2 and a layer of dysprosium metal 3 deposited on a surface of the magnetic body 2.

The magnetic body 2 comprises sintered grains 4 of a rare earth alloy. The grains 4 are shown as discrete granules with a boundary. Specifically, the bulk substance within the grains 4 comprises a Nd₂Fe₁₄B alloy. The grains 4 adjacent the deposited surface each have a shell layer 5 around their boundary. The shell layer 5 comprises diffused dysprosium which has substituted into the crystal lattice structure of the rare earth alloy. Although dysprosium can diffuse into the bulk of the crystal structure within the grains 4, careful control of the heat treatment conditions allow for diffusion to occur more readily at the grain boundaries. Specifically the shell layer 5 comprises a Dy₂Fe₁₄B or (Dy,Nd)₂Fe₁₄B alloy where the dysprosium has substituted into the neodymium alloy. The shell layer 5 of dysprosium containing alloy formed around each grain 4 has an approximate thickness of 0.5 µm.

The layer of dysprosium metal 3 is applied directly onto the magnetic body 2 using a cold spray technique. The layer 3 is shown to be uniform and to completely cover the top surface of the magnetic body 2. However, any surface of the magnetic body 2 may have a layer of dysprosium deposited onto it, and the layer 3 can be applied in a uniform or non-uniform manner. The thickness of the layer is shown schematically in the figures. A minimum thickness is desired to promote diffusion of dysprosium within or around the grains 4. However, a diminishing return of improved coercivity and magnetic properties is observed past a layer thickness of 5 µm.

A method of manufacturing the magnet 1 will now be described with reference to Figure 2. A magnetic body 2 containing grains of a Nd₂Fe₁₄B alloy 4 is provided. A surface of the magnetic body 2 is chosen to be coated in dysprosium. Dysprosium metal particles 6 are targeted, discharged and deposited onto the chosen surface. The conditions used for cold spray of other metal powders, such as copper and iron can be applied to the cold spraying of dysprosium metal particles. The deposited dysprosium metal rapidly forms a layer 3 on the targeted surface of the magnetic body 2.

Following the deposition of dysprosium, the magnet 1 is heat treated. During the heat treatment, the shell layer forms around the grains of the magnetic body 2. The heat treatment comprises a grain boundary diffusion process, such that the heat treatment causes dysprosium in the coating layer 3 to diffuse along the boundaries of grains 4 in the magnetic body 2 to form a shell layer 5 containing a dysprosium containing alloy 5.

The heat treatment follows the general method of heating the coated magnet 1 at a constant rate to an elevated first temperature and holding the magnet 1 at that elevated temperature for a time period of at least 6 hours. The first elevated temperature should be close to 1000 °C, ideally 900 °C. This temperature is hot enough to initiate and propagate the diffusion of dysprosium whilst avoiding sintering or melting of the magnetic grains 4.

The magnet 1 is then cooled at a controlled rate to a second elevated temperature which is lower than the first. The magnet 1 is held at this second elevated temperature for less time, around 30 minutes, before it is quenched to room temperature using a controlled cooling rate. The quenched magnet 1 exhibits improved magnetic properties, for example an increased coercivity.

The grains 4 comprise a Nd₂Fe₁₄B alloy. The grains can also comprise other magnetic rare earth alloys, such as those containing samarium, praseodymium or cerium, particularly SmCo₅ and Sm(Co, Fe, Cu, Zr)₇. The diffusion of the dysprosium layer 3 along the boundaries of the alloy grains 4 readily occurs for at least these rare earth alloys.

The grains 4 can be wholly coated in the shell layer 5, as shown in the figures. Alternatively, agglomerated grains 4 can be coated with a shell layer 5, such that the shell layer 5 only covers the exposed boundaries of the grains 4.

Further research has shown that rare earth magnetic metal terbium can also be used in a cold spray deposition process to create a rare earth magnet with improved coercivity.

## Claims

1. A method of manufacturing a magnet (1), the method comprising:
providing a magnetic body (2) containing grains (4) of a rare earth alloy; cold spray depositing a layer (3) of dysprosium or terbium onto the surface of the magnetic body (2); and
heat-treating the magnet (1).

2. The method in accordance with Claim 1, wherein heat-treating the magnet (1) comprises a grain boundary diffusion process.

3. The method in accordance with Claim 1 or 2, wherein heat-treating the magnet (1) comprises:
heating the magnet (1) to a first elevated temperature;
cooling the magnet (1) to second temperature; and
quenching the magnet (1) to room temperature.

4. The method in accordance with Claim 3, wherein the first elevated temperature is at least 900 °C.

5. The method in accordance with Claim 3 or 4, wherein the second temperature is at least 500 °C.

6. The method in accordance with any one of Claims 3 to 5, wherein the magnet (1) is held at the first elevated temperature for at least 6 hours.

7. The method in accordance with any one of Claims 3 to 6, wherein the magnet (1) is held at the second temperature for at least 0.5 hours.

8. The method in accordance with any one of Claims 1 to 7, wherein the rare earth alloy is a neodymium alloy.

9. A magnet (1) comprising a magnetic body (2) and a layer (3) of dysprosium or terbium ; wherein the magnetic body (2) contains grains (4) of a rare earth magnet alloy, **characterised in that** the layer (3) of dysprosium or terbium is deposited onto the surface of the magnetic body (2) by a cold spray process.

10. The magnet (1) in accordance with Claim 9, wherein the magnetic body (2) is sintered.

11. The magnet (1) in accordance with Claim 9 or Claim 10, wherein the rare earth alloy is a neodymium alloy.

12. The magnet (1) in accordance with any one of Claims 9 to 11, wherein an amount of dysprosium or terbium is diffused within the grains (4).

13. The magnet (1) in accordance with Claim 12, wherein the grains (4) contain an amount of diffused dysprosium or terbium of between 0.5 to 15 percent by weight.

14. The magnet (1) in accordance with Claims 12 or 13, wherein the dysprosium or terbium is diffused along the boundaries of the grains (4) to form a shell layer (5).

15. The magnet (1) in accordance with any one of Claims 9 to 14, wherein the deposition thickness of the layer (3) of dysprosium or terbium is between 1 to 5 µm.

## Patentansprüche

1. Verfahren zum Herstellen eines Magneten (1), wobei das Verfahren umfasst:
Bereitstellen eines magnetischen Körpers (2), der Körner (4) einer Seltenerdlegierung enthält;
kalte Sprühabscheidung einer Schicht (3) aus Dysprosium oder Terbium auf die Oberfläche des magnetischen Körpers (2); und
Wärmebehandeln des Magneten (1).

2. Verfahren nach Anspruch 1, wobei das Wärmebehandeln des Magneten (1) einen Korngrenzen-Diffusionsprozess umfasst.

3. Verfahren nach Anspruch 1 oder 2, wobei das Wärmebehandeln des Magneten (1) umfasst:
Erhitzen des Magneten (1) auf eine erste erhöhte Temperatur;
Kühlen des Magneten (1) auf eine zweite Temperatur; und
Abschrecken des Magneten (1) auf Raumtemperatur.

4. Verfahren nach Anspruch 3, wobei die erste erhöhte Temperatur mindestens 900 °C beträgt.

5. Verfahren nach Anspruch 3 oder 4, wobei die zweite Temperatur mindestens 500 °C beträgt.

6. Verfahren nach einem der Ansprüche 3 bis 5, wobei der Magnet (1) für mindestens 6 Stunden bei der ersten erhöhten Temperatur gehalten wird.

7. Verfahren nach einem der Ansprüche 3 bis 6, wobei der Magnet (1) für mindestens 0,5 Stunden bei der zweiten Temperatur gehalten wird.

8. Verfahren nach einem der Ansprüche 1 bis 7, wobei die Seltenerdlegierung eine Neodymlegierung ist.

9. Magnet (1) umfassend einen magnetischen Körper (2) und eine Schicht (3) aus Dysprosium oder Terbium; wobei der magnetische Körper (2) Körner (4) einer Seltenerdmagnetlegierung enthält,
**dadurch gekennzeichnet, dass**
die Schicht (3) aus Dysprosium oder Terbium durch einen kalten Sprühprozess auf der Oberfläche des magnetischen Körpers (2) abgeschieden wird.

10. Magnet (1) nach Anspruch 9, wobei der magnetische Körper (2) gesintert wird.

11. Magnet (1) nach Anspruch 9 oder Anspruch 10, wobei die Seltenerdlegierung eine Neodymlegierung ist.

12. Magnet (1) nach einem der Ansprüche 9 bis 11, wobei eine Menge des Dysprosium oder Terbium innerhalb der Körner (4) diffundiert wird.

13. Magnet (1) nach Anspruch 12, wobei die Körner (4) eine Menge an diffundiertem Dysprosium oder Terbium zwischen 0,5 und 15 Gew.-% enthalten.

14. Magnet (1) nach Ansprüchen 12 oder 13, wobei das Dysprosium oder Terbium entlang der Grenzen der Körner (4) diffundiert wird, um eine Hüllschicht (5) zu bilden.

15. Magnet (1) nach einem der Ansprüche 9 bis 14, wobei die Abscheidungsdicke der Schicht (3) aus Dysprosium oder Terbium zwischen 1 und 5 µm beträgt.

## Revendications

1. Procédé de fabrication d'un aimant (1), le procédé comprenant :
l'obtention d'un corps magnétique (2) contenant des grains (4) d'un alliage de terres rares ;
le dépôt par projection à froid d'une couche (3) de dysprosium ou de terbium sur la surface du corps magnétique (2) ; et
le traitement thermique de l'aimant (1).

2. Procédé selon la revendication 1, dans lequel le traitement thermique de l'aimant (1) comprend un procédé de diffusion aux joints de grains.

3. Procédé selon la revendication 1 ou 2, dans lequel le traitement thermique de l'aimant (1) comprend :
le chauffage de l'aimant (1) jusqu'à une première température élevée ;
le refroidissement de l'aimant (1) jusqu'à une deuxième température ; et
la trempe de l'aimant (1) jusqu'à la température ambiante.

4. Procédé selon la revendication 3, dans lequel la première température élevée est d'au moins 900 °C.

5. Procédé selon la revendication 3 ou 4 dans lequel la deuxième température est d'au moins 500 °C.

6. Procédé selon l'une quelconque des revendications 3 à 5, dans lequel l'aimant (1) est maintenu à la première température élevée pendant au moins 6 heures.

7. Procédé selon l'une quelconque des revendications 3 à 6, dans lequel l'aimant (1) est maintenu à la deuxième température pendant au moins 0,5 heure.

8. Procédé selon l'une quelconque des revendications 1 à 7, dans lequel l'alliage de terres rares est un alliage de néodyme.

9. Aimant (1) comprenant un corps magnétique (2) et une couche (3) de dysprosium ou de terbium, le corps magnétique (2) contenant des grains (4) d'un alliage de terres rares pour aimants,
**caractérisé en ce que**
la couche (3) de dysprosium ou de terbium est déposée sur la surface du corps magnétique (2) par un procédé de projection à froid.

10. Aimant (1) selon la revendication 9, dans lequel le corps magnétique (2) est fritté.

11. Aimant (1) selon la revendication 9 ou la revendication 10, dans lequel l'alliage de terres rares est un alliage de néodyme.

12. Aimant (1) selon l'une quelconque des revendications 9 à 11, dans lequel une quantité de dysprosium ou de terbium est diffusée à l'intérieur des grains (4).

13. Aimant (1) selon la revendication 12, dans lequel les grains (4) contiennent une quantité de dysprosium ou de terbium diffusé comprise entre 0,5 et 15 pour cent en poids.

14. Aimant (1) selon la revendication 12 ou 13, dans lequel le dysprosium ou le terbium est diffusé le long des joints des grains (4) pour former une couche de coquille (5).

15. Aimant (1) selon l'une quelconque des revendications 9 à 14, dans lequel l'épaisseur de dépôt de la couche (3) de dysprosium ou de terbium se situe entre 1 et 5 µm.
